# EUROPEAN PATENT SPECIFICATION

(11) **EP 1 890 824 B1**
(45) Date of publication and mention of the grant of the patent: **05.10.2016**
(21) Application number: 06757802.1
(22) Date of filing: 16.06.2006
(51) Int. Cl.: B05D 7/00, B05D 3/06, B05D 1/02

(54) **METHOD FOR APPLYING A LAYER TO A SURFACE, AS WELL AS AN ASSEMBLY AND A DECORATIVE PANEL**
VERFAHREN ZUM AUFBRINGEN EINER SCHICHT AUF EINE FLÄCHE SOWIE ANORDNUNG UND ZIERPLATTE
PROCEDE D'APPLICATION DE COUCHE SUR UNE SURFACE, ENSEMBLE ET PANNEAU DECORATIF

(30) Priority: 17.06.2005 NL 1029274
(43) Date of publication of application: 27.02.2008
(73) Proprietor: Trespa International B.V., 6002 SM Weert (NL)
(72) Inventor: VONCKEN, Hendrikus, Hubertus, Gerardus, NL-6181 ES Elsloo (NL); VAN DE WALL, Wilhelmus, Josephus, Alex, NL-5591 CS Heeze (NL)
(74) Representative: Algemeen Octrooi- en Merkenbureau B.V.
(86) International application number: PCT/NL2006/000297
(87) International publication number: WO 2006/135234

(56) References cited:
- EP-A- 0 724 914
- WO-A-92/21450
- WO-A-03/064061
- US-A- 5 194 293
- US-B1- 6 528 126
- US-B1- 6 677 045

## Description

Method for applying a layer to a surface, as well as an assembly and a decorative panel.

The present invention relates to a method for applying a layer to a surface. The present invention furthermore relates to an assembly consisting of a layer applied to a surface, and to a decorative panel built up of a core and a decorative layer on one or on both sides of the core.

From US patent No. 6,185,840 a method is known wherein a radiation-curable layer is applied to a substrate, for example paper, glass, plastics, wood or metal. The layer thus applied is passed through a curing unit, which uses ultraviolet light for the curing step, whilst the space in which the curing step is carried out is flushed with a gas. The method that is known therefrom in fact comprises two steps, viz. a first step, in which the applied layer, which generally is heat-sensitive and has a thickness of 10-50 µm, must be cooled during the UV radiation. The second step can be considered as a drying/curing operation in a specific atmosphere, for example an inert gas, in particular nitrogen or carbon dioxide. The inert atmosphere in particular functions to prevent the chemical reactions being adversely affected, so that a good bond and good surface properties are obtained.

European patent application No. 0 724 914 relates to a method for the continuous painting of moving elements, in particular rod-shaped wooden elements, wherein, after the application of a first layer of paint to the element, the layer of paint thus applied is removed by brushing, after which a second layer of paint is applied, and the drying thereof is carried out by means of ultraviolet radiation.

European patent application No. 1 157 750 relates to a method for coating the internal surface of a polyethylene container with a radiation-curable epoxy-based polymeric composition, using electromagnetic radiation.

US patent No. 6,677,045 relates to a multilayer coating comprising a basecoat layer and a topcoat layer, wherein a basecoat layer is applied to a substrate and heated to a temperature of maximally 100 °C, after which a topcoat is applied to said basecoat layer, followed by radiation curing. Although the basecoat layer is not fully cured after said thermal treatment, it cannot be considered as a fluid layer.

International application WO 03/064061 relates to a process for the application of a coating to a substrate, wherein the substrate is pre-treated by means of a low-temperature plasma, a corona discharge or a flame, after which a coating is applied to the substrate thus pre-treated, which coating is subsequently dried by means of electromagnetic waves.

US patent No. 6,528,126 relates to a process for the application of a multilayer coating to a (possibly precoated) substrate, wherein a coating is applied to the substrate, to which a topcoat is applied, after which at least one of the layers thus applied is alternately irradiated with UV radiation and IR radiation, using a radiation source comprising UV radiation as well as IR radiation, which radiation lasts at least 30 seconds.

The object of the present invention is to apply a thin layer to a surface whilst effecting a good bond of the thin layer to the surface.

Another object of the invention is to apply a thin layer to a surface, wherein the thin layer penetrates the surface by diffusion, in such a manner that the functionality of the thin layer is retained.

Yet another object of the invention is to make it possible to influence the functionality of the thin layer as needed.

The method as referred to in introductory paragraph is characterised in that layer said method comprises the following steps:
i) the provision of a fluid layer comprising radiation curable components yet to be cured, said layer being present on a substrate,
ii) the application of said top layer on top of said fluid layer comprising radiation curable components by means of an aerosol comprising active components,
iii) the application of radiation in a radiation unit, viz. a UV unit or an EB (electron beam) unit, on the assembly obtained after step ii), wherein polymerization of said fluid layer comprising radiation curable components takes place, and as a result of the exothermic reaction heat that is released during said polymerization evaporation of the liquid components present in said top layer takes place resulting in a said active components containing top layer having a thickness of 1-200 nm.

The use of an aerosol makes it possible to apply very thin layers to the surface, in which connection the aerosol technique must be considered as a flow of droplets in a gas phase, with the diameter of the droplets generally being significantly smaller than 100 µm. Such droplets may also contain one or more solids. It is also possible, however, to dissolve solids in a solvent first and then convert the composition thus obtained into an aerosol. Coatings differing from each other as regards quality and functionality can be obtained by using a special selection of the liquid-gas composition of the aerosol. Thus it is possible in the present invention to adapt the functionality of the layer applied as an aerosol, in which connection in particular a specific degree of gloss, antistatic properties, a high scratch resistance, antibacterial properties and self-cleaning properties must be considered. A certain degree of mixing will take place at the interface of the aerosol still fluid and that curing of said surface must take place yet. Mixing is such that the functionality of the layer applied as an aerosol is retained. In the present invention, the surface and the layer that has been applied thereto as an aerosol are cured in a single radiation step, with no forced drying step or other intermediate processing steps being required.

To effect a good bond between the layer applied as an aerosol and the surface it is desirable to apply for the aerosol to a fluid layer yet to be cured by radiation, in which connection it is in particular desirable to subject the assembly of aerosol and layer yet to be cured by radiation to a follow-up treatment with radiation, in particular electron radiation and/or UV radiation. Thus a good bond between the aerosol layer and the fluid surface is realised. The curing process is carried out in fractions of seconds. Furthermore, there is no need for combinations of radiation sources.

The aerosol formulation, which may in particular be a water-based or a solvent-containing aerosol, consists on the one hand of one or more active components which provide the bond and the compatibility with the surface and on the other hand of components that provide the eventual functionality of the surface of the layer applied as an aerosol. In a special embodiment of the present invention, it is preferable to use components which combine the two properties, for example molecules comprising a group having surface functionality, such as quaternary ammonium salts, and a group that can be cured by radiation, such as acrylate. In a specific embodiment, the aerosol preferably contains only one or more active components, without additional solvents, such as water or organic solvents, being used.

As a result of the use of water and/or solvents in the aerosol formulation it has appeared to be possible to apply a relatively thick layer to the surface, which layer can more or less flow together with the still fluid surface to form a closed film. Part of the water and/or the solvents will evaporate upon transfer of the combination of surface and layer applied as an aerosol thus effected to a radiation unit, viz. a UV unit or an EB (electron beam) unit. Complete evaporation generally takes place as a result of the exothermic reaction heat that is released during the polymerisation step in the radiation unit. After evaporation, the final layer thickness of the layer applied as an aerosol is reached.

Using the present method, a layer thickness of 1-200 nm after curing of the layer applied as an aerosol can be realised, with the thickness of the radiation-curable layer of the surface being 4-100 µm.

In a special embodiment, the fluid surface is preferably present on a substrate, in particular a cellulose-containing material impregnated with a curable resin. Impregnated paper, in particular of one or more kraft papers impregnated with a phenol resin, can be mentioned as a suitable substrate.

The aerosol to be used in the present invention preferably contains components to be cured by means of electron radiation and/or UV radiation, and it may be a water-based or a solvent-containing formulation.

In the present invention one or more functional components selected from the group consisting of bactericides, brighteners, scratch resistance enhancers, matting agents, antistatics, surface tension modifiers, algicides, anti-graffiti agents, surface-cleaning agents, pigments, friction-influencing agents and fire retardants, may be added to the aerosol.

The present invention further relates to an assembly comprising a layer present on a surface, which is characterised in that said layer is a layer applied as an aerosol and that the surface is a radiation-cured layer.

The thickness of the layer applied as an aerosol in the present assembly is 1-200 nm after curing, with the thickness of the radiation-cured layer being 4-100 µm.

In a special embodiment, one or more components selected from the group consisting of bactericides, brighteners, scratch resistance enhancers, matting agents, antistatics, surface tension modifiers, algicides, anti-graffiti agents, surface-cleaning agents, pigments, friction-influencing agents and fire retardants is (are) preferably contained in the layer applied as an aerosol.

In a special embodiment of the present assembly, the surface, which is a radiation-cured layer, is present on a substrate, preferably a cellulose-containing material impregnated with a curable resin, in particular an impregnated paper, such as a kraft paper impregnated with a phenol resin, or a number of such kraft paper layers.

The present assembly is in particular suitable for being used in a decorative panel, which decorative panel is built up of a core provided with one or more decorative layers on one or on both sides thereof, wherein the present assembly is used as a decorative layer. The core that is used may in particular be composed of one or more resin-impregnated, cellulose-containing layers.

Using the present method, wherein a so-called aerosol deposition is carried out in combination with a layer yet to be cured by radiation, it is possible to apply a very thin layer to a fluid surface, in particular a previously applied coating, wherein a durable bond between the layer and the surface is effected as a result of the rapid curing that takes place when a radiation-curable crosslinking process is carried out. Using the present method it is in particular possible to adjust the functionality of the layer applied as an aerosol, in particular the upper layer, according to specific objectives.

The present invention will now be explained by means of a number of examples, in which connection it should be noted, however, that the present invention is by no means limited to such special examples.

### Examples.

A coating of a radiation-curable coating consisting of an acrylate groups-containing oligomer (65%) diluted with HDDA to a viscosity of 2000 mPas was applied to PVC in a thickness about 30 µm by means of a film applicator. The same radiation-curable coating was applied to a partially cured coating, which coating was in turn applied to a paper impregnated with a phenol resin.

A water-based formulation was applied as an aerosol to the still fluid acrylate groups-containing coating by means of an airbrush gun. The intention was to obtain a closed film layer. The film layer applied as an aerosol was closed at 1-10 g/m² of wet film. The layer thickness required in order to have water droplets flow together into a closed film appeared to depend on the surface tension of the aqueous formulation. Said surface tension was set by adding a surfactant. An amount of 0.2 wt.% of softanol 70 was added to the water for setting the surface tension.

It was established that the kinetic energy of the droplets to be sprayed must not be too large, because they will interfere with the wet underlying film layer in that case and the droplets are prevented from flowing together if they impact too deep into the wet layer. The impact can be reduced by using small droplets with low impact velocities.

The samples with the still fluid radiation-curable coating with the water-based formulation applied as an aerosol present thereon were transported to an electron beam radiation source, after which the entire system was polymerised, using an acceleration voltage of 150 kV and a surface dosage of 60 kGray.

The water in the water-based formulation largely evaporated during transport to the radiation source and during radiation with electrons.

A properly cured surface film had formed after the radiation step. No harmful effects of the applied water could be observed.

The active components in the water-based formulation are present in a very thin layer on the surface, i.e. a radiation curable-coating, therefore.

Since the active components in the water-based formulation either contain radiation-curable groups or are mixed with radiation-curable components or are readily compatible with the still fluid surface, the active components are irreversibly bound to the radiation-curable coating to which the water-based formulation had been applied.

The following effects were measured:
**Surface tension of samples on PVC, measured by means of the ink technique:** Reference sample
99.8% water, 0.2% softenol 70 35 mN/m

### Sample A

95.8% water, 2% Uvecoat 7177, 2% 2-acryloyloxy ethyl trimethyl-ammoniumchloride, 0.2% softenol 70 52 mN/m

### Surface resistivity, Ohm/square

### Reference sample

99.8% water, 0.2% softenol 70 >10 E 12.5 Ohm/square

### Sample B

94.8% water, 3% Uvecoat 7177, 2% biocoat 220, 0.2% softenol 70
10 E 10 Ohm/square

### Cleanability

### Reference sample

99.8% water, 0.2% softenol 70
Adequate and complete removal of Edding 3000 permanent marker

### Sample C

97.8% water, 2% 2,2,3,3,4,4,4-heptafluorobutylacrylate,
0.2% softenol 70
Simple and complete removal of Edding 3000 permanent marker

### HPL

Plates having a thickness of 6 mm were pressed from the samples applied to phenol-impregnated paper, using techniques that are known in the HPL industry (EN 438). Upon measurement, these plates appeared to have the following properties:

### Surface resistivity, Ohm/square

### Reference sample

99.8% water, 0.2% softenol 70 >10 E 12.5 Ohm/square

### Sample D

97.8% water, 2% 2-acryloyloxy ethyltrimethyl ammonium chloride, 0.2% softanol 70
10 E 9 Ohm/square

### Graffity removal: removal of Edding 3000 permanent marker

### Reference sample

99.8% water, 0.2% softenol 70 Adequate and complete cleaning

### Sample C

97.8% water, 2% 2,2,3,3,4,4,4-heptafluorobutylacrylate,
0.2% softenol 70
Simple and complete removal of Edding 3000 permanent marker

### Activity van E. Coli.

The aforesaid reference sample and Sample B were examined for antibacterial properties, using the JIS Z 2801:2000 method. As a pre-treatment, the samples were subjected to a thorough cleaning operation involving rinsing in hot water and ethanol, with the layer applied as an aerosol in Sample B not exhibiting any delamination.

The activity of E.coli amounted to t = 0, 1.2•10⁴ for the reference sample, and decreased to a value of 1.1•10⁴ after 1 hour. The values measured for Sample B were 1.2•10⁴ and 2.3•10³, respectively, which latter value shows a distinct antibacterial activity.

From the above measuring data it is apparent that samples A-D can be given specific functionalities, as a result of which the properties of the respective samples A-D are affected in comparison with the reference sample, which does not comprise such components that influence the functionality. The use of the aerosol formulation has furthermore shown that it is possible to apply uniformly distributed thin layers to a surface.

## Claims

1. A method for functionalising a layer comprising radiation curable components by depositing a top layer on top of said layer, **characterized in that**, said method comprises the following steps:
i) the provision of a fluid layer comprising radiation curable components yet to be cured, said layer being present on a substrate,
ii) the application of said top layer on top of said fluid layer comprising radiation curable components by means of an aerosol comprising active component.
iii) the application of radiation in a radiation unit viz, a UV unit or an EB (electron beam) unit, on the components, assembly obtained after step ii), wherein polymerization of said fluid layer comprising radiation curable components takes place, and as a result of the exothermic reaction heat that is released during said polymerization evaporation of the liquid components present in said top layer takes place resulting in a said active components containing top layer having a thickness of 1-200 nm.

2. A method according to claim 1, **characterised in that** the thickness of the layer comprising radiation curable components is 4-100 µm.

3. A method according to claim 1, **characterised in that** said substrate is a cellulose-containing material impregnated with a curable resin.

4. A method according to claim 3, **characterised in that** the substrate is an impregnated paper.

5. A method according to claim 3, **characterised in that** said substrate is a kraft paper impregnated with a phenol resin.

6. A method according to any one or more of the preceding claims, **characterised in that** the aerosol contains one or more solvents.

7. A method according to claim 6, **characterised in that** the aerosol is water-based.

8. A method according to any one or more of the preceding claims, **characterised in that** the aerosol contains electron radiation and/or UV radiation curable components.

9. A method according to any one or more of the preceding claims, **characterised in that** said active components present in said aerosol are selected from the group consisting of bactericides, brighteners, scratch resistance enhancers, matting agents, antistatics, surface tension modifiers, algicides, anti-graffiti agents, surface-cleaning agents, pigments, friction-influencing agents and fire retardants.

10. A method according to any one or more of the preceding claims, **characterised in that** said aerosol is a flow of droplets in a gas phase, with the diameter of the droplets being < 100 µm, wherein said droplets contain active components.

11. A method according to any one or more of the preceding claims, **characterised in that** step iii) is a single radiation step, with no forced drying step or other intermediate processing steps being required.

12. A method according to any one or more of the preceding claims, **characterised in that** said active components are molecules comprising a group having surface functionality and a group that can be cured by radiation.

13. A method according to claim 12, **characterised in that** as a group that can be cured by radiation an acrylate is used.

14. An assembly comprising a layer comprising radiation curable components on a substrate, **characterised in that** on top of said layer is a top layer applied as an aerosol, said top layer having a thickness of 1-200 nm.

15. An assembly according to claim 14, **characterised in that** the thickness of the layer comprising radiation curable components is 4-100 µm.

16. An assembly according to any one or more of the claims 14 or 15, **characterised in that** one or more components selected from the group consisting of bactericides, brighteners, scratch resistance enhancers, matting agents, antistatics, surface tension modifiers, algicides, anti-graffiti agents, surface-cleaning agents, pigments, friction-influencing agents and fire retardants is (are) contained in said top layer.

17. An assembly according to claim 14, **characterised in that** said substrate is a cellulose-containing material impregnated with a curable resin.

18. An assembly according to claim 17, **characterised in that** said substrate is an impregnated paper.

19. An assembly according to claim 18, **characterised in that** said substrate is a kraft paper impregnated with a phenol resin.

20. A decorative panel built up of a core and a decorative layer on one or on both sides of the core, **characterised in that** an assembly according to any one of the claims 14-19 has been used as the decorative layer.

21. A decorative panel according to claim 20, **characterised in that** said core is composed of one or more resin-impregnated, cellulose-containing layers.

## Patentansprüche

1. Verfahren zum Funktionalisieren einer Schicht mit strahlungshärtbaren Komponenten durch Abscheiden einer Deckschicht auf der Schicht, **dadurch gekennzeichnet, dass** das Verfahren die folgenden Schritte umfasst:
i) das Bereitstellen einer Fluidschicht mit noch zu härtenden strahlungshärtbaren Komponenten, wobei sich die Schicht auf einem Substrat befindet,
ii) das Aufbringen der Deckschicht auf die Fluidschicht mit strahlungshärtbaren Komponenten mittels eines eine aktive Komponente umfassenden Aerosols,
iii) das Applizieren von Strahlung in einer Strahlungseinheit, d.h. einer UV-Einheit oder einer ES (Elektronenstrahl)-Einheit, auf das nach Schritt ii) erhaltene Aggregat, wobei eine Polymerisation der Fluidschicht mit strahlungshärtbaren Komponenten erfolgt und als Folge der exothermen Reaktionswärme, die während der Polymerisation frei wird, eine Verdampfung der in der Deckschicht vorhandenen flüssigen Komponenten erfolgt, was dazu führt, dass die aktive Komponenten enthaltende Deckschicht eine Dicke von 1-200 nm aufweist.

2. Verfahren nach Anspruch 1, **dadurch gekennzeichnet, dass** die Dicke der Schicht mit strahlungshärtbaren Komponenten 4-100 µm beträgt.

3. Verfahren nach Anspruch 1, **dadurch gekennzeichnet, dass** das Substrat ein mit einem härtbaren Harz imprägniertes cellulosehaltiges Material ist.

4. Verfahren nach Anspruch 3, **dadurch gekennzeichnet, dass** das Substrat ein imprägniertes Papier ist.

5. Verfahren nach Anspruch 3, **dadurch gekennzeichnet, dass** das Substrat ein mit einem Phenolharz imprägniertes Kraftpapier ist.

6. Verfahren nach einem oder mehreren der vorangegangenen Ansprüche, **dadurch gekennzeichnet, dass** das Aerosol ein oder mehrere Lösungsmittel enthält.

7. Verfahren nach Anspruch 6, **dadurch gekennzeichnet, dass** das Aerosol auf Wasser basiert.

8. Verfahren nach einem oder mehreren der vorangegangenen Ansprüche, **dadurch gekennzeichnet, dass** das Aerosol durch Elektronenstrahlung und/oder UV-Strahlung härtbare Komponenten enthält.

9. Verfahren nach einem oder mehreren der vorangegangenen Ansprüche, **dadurch gekennzeichnet, dass** die in dem Aerosol vorliegenden aktiven Komponenten aus der Gruppe bestehend aus Bakteriziden, Aufhellern, Mitteln zur Verbesserung der Kratzfestigkeit, Mattierungsmitteln, Antistatika, Mitteln zur Modifizierung der Oberflächenspannung, Algiziden, Antigraffitimitteln, Mitteln zur Oberflächenreinigung, Pigmenten, Mitteln zur Beeinflussung der Reibung und Brandschutzmitteln ausgewählt sind.

10. Verfahren nach einem oder mehreren der vorangegangenen Ansprüche, **dadurch gekennzeichnet, dass** das Aerosol ein Tröpfchenstrom in einer Gasphase ist, wobei der Durchmesser der Tröpfchen < 100 µm beträgt, wobei die Tröpfchen aktive Komponenten enthalten.

11. Verfahren nach einem oder mehreren der vorangegangenen Ansprüche, **dadurch gekennzeichnet, dass** Schritt iii) ein alleiniger Bestrahlungsschritt ist, ohne dass ein erzwungener Trocknungsschritt oder andere Bearbeitungszwischenschritte erforderlich sind.

12. Verfahren nach einem oder mehreren der vorangegangenen Ansprüche, **dadurch gekennzeichnet, dass** die aktiven Komponenten Moleküle sind, die eine Gruppe mit einer Oberflächenfunktionalität und eine durch Strahlung härtbare Gruppe umfassen.

13. Verfahren nach Anspruch 12, **dadurch gekennzeichnet, dass** als eine durch Strahlung härtbare Gruppe ein Acrylat verwendet wird.

14. Aggregat mit einer strahlungshärtbare Komponenten umfassenden Schicht auf einem Substrat, **dadurch gekennzeichnet, dass** sich auf der Schicht eine als Aerosol aufgebrachte Deckschicht befindet, wobei die Deckschicht eine Dicke von 1-200 nm aufweist.

15. Aggregat nach Anspruch 14, **dadurch gekennzeichnet, dass** die Dicke der strahlungshärtbare Komponenten umfassenden Schicht 4-100 µm beträgt.

16. Aggregat nach einem oder mehreren der Ansprüche 14 oder 15, **dadurch gekennzeichnet, dass** eine oder mehrere Komponenten, ausgewählt aus der Gruppe bestehend aus Bakteriziden, Aufhellern, Mitteln zur Verbesserung der Kratzfestigkeit, Mattierungsmitteln, Antistatika, Mitteln zur Modifizierung der Oberflächenspannung, Algiziden, Antigraffitimitteln, Mitteln zur Oberflächenreinigung, Pigmenten, Mitteln zur Beeinflussung der Reibung und Brandschutzmitteln, in der Deckschicht enthalten ist/sind.

17. Aggregat nach Anspruch 14, **dadurch gekennzeichnet, dass** das Substrat ein mit einem härtbaren Harz imprägniertes cellulosehaltiges Material ist.

18. Aggregat nach Anspruch 17, **dadurch gekennzeichnet, dass** das Substrat ein imprägniertes Papier ist.

19. Aggregat nach Anspruch 18, **dadurch gekennzeichnet, dass** das Substrat ein mit einem Phenolharz imprägniertes Kraftpapier ist.

20. Dekorpaneel, das aus einem Kern und einer Dekorschicht auf einer oder beiden Seiten des Kerns aufgebaut ist, **dadurch gekennzeichnet, dass** ein Aggregat nach einem der Ansprüche 14 bis 19 als Dekorschicht verwendet wurde.

21. Dekorpaneel nach Anspruch 20, **dadurch gekennzeichnet, dass** der Kern aus einer oder mehreren mit Harz imprägnierten, cellulosehaltigen Schichten zusammengesetzt ist.

## Revendications

1. Procédé de fonctionnalisation d'une couche comprenant des composants durcissables par rayonnement par dépôt d'une couche supérieure au-dessus de ladite couche, **caractérisé en ce que** ledit procédé comprend les étapes suivantes :
i) la fourniture d'une couche de fluide comprenant des composants durcissables par rayonnement qui n'est pas encore durcie, ladite couche étant présente sur un substrat,
ii) l'application de ladite couche supérieure au-dessus de ladite couche de fluide comprenant des composants durcissables par rayonnement au moyen d'un aérosol comprenant un composant actif.
iii) l'application d'un rayonnement dans une unité de rayonnement, à savoir, une unité UV ou une unité EB (à faisceau électronique), sur l'ensemble obtenu après l'étape ii), où la polymérisation de ladite couche de fluide comprenant des composants durcissables par rayonnement a lieu, et en raison de la chaleur de réaction exothermique qui est libérée durant ladite polymérisation, une évaporation des composants liquides présents dans ladite couche supérieure a lieu, donnant lieu à ladite couche supérieure contenant des composants actifs ayant une épaisseur de 1 à 200 nm.

2. Procédé selon la revendication 1, **caractérisé en ce que** l'épaisseur de la couche comprenant des composants durcissables par rayonnement est de 4 à 100 µm.

3. Procédé selon la revendication 1, **caractérisé en ce que** ledit substrat est un matériau contenant de la cellulose imprégné d'une résine durcissable.

4. Procédé selon la revendication 3, **caractérisé en ce que** le substrat est un papier imprégné.

5. Procédé selon la revendication 3, **caractérisé en ce que** ledit substrat est un papier kraft imprégné d'une résine phénolique.

6. Procédé selon l'une quelconque ou plusieurs des revendications précédentes, **caractérisé en ce que** l'aérosol contient un ou plusieurs solvant(s).

7. Procédé selon la revendication 6, **caractérisé en ce que** l'aérosol est à base d'eau.

8. Procédé selon l'une quelconque ou plusieurs des revendications précédentes, **caractérisé en ce que** l'aérosol contient des composants durcissables par rayonnement électronique et/ou par rayonnement UV.

9. Procédé selon l'une quelconque ou plusieurs des revendications précédentes, **caractérisé en ce que** lesdits composants actifs présents dans ledit aérosol sont choisis dans le groupe constitué par des bactéricides, des azurants optiques, des agents améliorant la résistance à la rayure, des agents de matité, des agents antistatiques, des modificateurs de tension superficielle, des algicides, des agents anti-graffitis, des agents de nettoyage de surface, des pigments, des agents influant sur le frottement et des agents ignifuges.

10. Procédé selon l'une quelconque ou plusieurs des revendications précédentes, **caractérisé en ce que** ledit aérosol est un écoulement de gouttelettes dans une phase gazeuse, le diamètre des gouttelettes étant < 100 µm, où lesdites gouttelettes contiennent des composants actifs.

11. Procédé selon l'une quelconque ou plusieurs des revendications précédentes, **caractérisé en ce que** l'étape iii) est une seule étape de rayonnement, sans qu'une étape de séchage forcé ou autres étapes de traitement intermédiaires ne soit/soient nécessaire(s).

12. Procédé selon l'une quelconque ou plusieurs des revendications précédentes, **caractérisé en ce que** lesdits composants actifs sont des molécules comprenant un groupe ayant une fonctionnalité de surface et un groupe qui peut être durci par rayonnement.

13. Procédé selon la revendication 12, **caractérisé en ce qu'**un acrylate est utilisé en tant que groupe qui peut être durci par rayonnement.

14. Ensemble comprenant une couche qui comprend des composants durcissables par rayonnement sur un substrat, **caractérisé en ce qu'**une couche supérieure est appliquée en tant qu'aérosol au-dessus de ladite couche, ladite couche supérieure ayant une épaisseur allant de 1 à 200 nm.

15. Ensemble selon la revendication 14, **caractérisé en ce que** l'épaisseur de la couche comprenant des composants durcissables par rayonnement est de 4 à 100 µm.

16. Ensemble selon l'une quelconque ou des plusieurs revendications 14 ou 15, **caractérisé en ce qu'**un ou plusieurs composant(s) choisi(s) dans le groupe constitué par des bactéricides, des azurants optiques, des agents améliorant la résistance à la rayure, des agents de matité, des agents antistatiques, des modificateurs de tension superficielle, des algicides, des agents anti-graffitis, des agents de nettoyage de surface, des pigments, des agents influant sur le frottement et des agents ignifuges est/sont contenu(s) dans ladite couche supérieure.

17. Ensemble selon la revendication 14, **caractérisé en ce que** ledit substrat est un matériau contenant de la cellulose imprégné d'une résine durcissable.

18. Ensemble selon la revendication 17, **caractérisé en ce que** ledit substrat est un papier imprégné.

19. Ensemble selon la revendication 18, **caractérisé en ce que** ledit substrat est un papier kraft imprégné d'une résine phénolique.

20. Tableau décoratif formé d'une partie centrale et d'une couche décorative sur un ou sur les deux côtés de la partie centrale, **caractérisé en ce qu'**un ensemble selon l'une quelconque des revendications 14 à 19 a été utilisé comme étant la couche décorative.

21. Panneau décoratif selon la revendication 20, **caractérisé en ce que** ladite partie centrale est composée d'une ou de plusieurs couche(s) contenant de la cellulose, imprégnée(s) de résine.
